

# UNITED STATES PATENT OFFICE.

EUGENE DU PONT, OF WILMINGTON, DELAWARE.

## EXPLOSIVE COMPOUND.

SPECIFICATION forming part of Letters Patent No. 352,611, dated November 16, 1886.

Application filed June 16, 1886. Serial No. 205,362. (No specimens.)

*To all whom it may concern:*

Be it known that I, EUGENE DU PONT, a citizen of the United States, residing at Wilmington, county of New Castle, and State of Delaware, have invented a certain new and useful Improvement in Explosive Compounds; and I hereby declare that the following is a full, clear, and exact description of the same.

My invention consists in the use, in explosive compounds, of wood slightly changed in its chemical formula by the application of heat for the two purposes of increasing the ballistic force of the powder and of controlling the rate of combustion so as to adapt it for use in heavy charges behind projectiles of great weight, or to lighter charges in medium-sized guns. With this end in view I replace (either wholly or partially, as desired) the charcoal which is used in the composition of ordinary gunpowder, with the requisite amount of wood slightly changed in its chemical formula by having been subjected to heat, or baked, as hereinafter described.

I have found that branch-willow wood is well adapted to the purpose; but any suitable wood for making gunpowder-charcoal may be used.

I subject the wood to a gentle heat, (either in a retort over a slow fire or by the application of superheated steam in a suitable vessel,) gradually raising the temperature to about 450° Fahrenheit, at which the heat is maintained for about two hours, (this would be for three-fourths of a cord of willow,) the entire time consumed in the baking being about eight hours, six hours being consumed in obtaining the proper temperature. The limits of temperature at which the baking should cease (as far as I am now aware) to secure good results are 300° Fahrenheit, and 450° Fahrenheit, the lower temperature making the wood less rapidly combustible, and the higher securing a more combustible wood. The process of heating the wood, as described, should cease before the wood is transformed into red charcoal, which is useless for my purpose, as red charcoal has entirely lost the fibrous character of the wood, while in the wood which I use in the present invention the fiber is still undestroyed; and it is by breaking the wood and examining if the fiber has been destroyed that I am able to determine the point at which the baking should cease. 450° Fahrenheit is a tem-

perature high enough to transform the wood into red charcoal, if maintained for a sufficient length of time; but I remove the wood before 55 such transformation takes place.

My baked wood differs from red charcoal not only in its physical character by retaining its fiber, but also in its chemical formula. Red charcoal is considered to contain about 72.64 60 per cent. of carbon, 4.71 per cent. of hydrogen, 20.08 per cent. of oxygen, and 0.57 per cent. of ash. Although not being a definite chemical compound, but being produced by partial decomposition, it will vary slightly in 65 its formula. This also applies to my baked wood, which may vary even more than from 47.51 per cent. of carbon, 6.12 per cent. of hydrogen, 46.29 per cent. of oxygen, and 0.08 per cent. of ash, to 51.82 per cent. of carbon, 3.99 70 per cent. of hydrogen, 43.94 per cent. of oxygen, and 0.22 per cent. of ash; but, as will be seen, it has much less carbon than red charcoal, and still less than black charcoal. The carbon in my baked wood also retains to a cer- 75 tain extent, after being ground fine, its cellular form, and combines with the liberated oxygen from the saltpeter more readily than other forms of carbon—for instance, stone-coal or lamp-black.

80

The greater proportion of oxygen and hydrogen in my baked wood than in charcoal is of very great importance to the ballistic effect of the powder. The theory of their action, as proved by experiment, is as follows: The temperature, after ignition of the charge in the gun, reaches 4,000° Fahrenheit, a degree of heat too high to permit the oxygen and hydrogen to combine to form water, and they therefore must remain uncombined until, by 85 the expansion due to the motion of the projectile toward the muzzle, these gases are cooled sufficiently to permit their union. When this takes place, a very large amount of heat is disengaged, which expands again the 90 steam and other gases formed by the combustion of the powder. The pressure thus sus- tained while the projectile is in the gun insures a high velocity and a low pressure, be- cause all the atoms of the powder cannot form 100 new combinations at the time of ignition, but part of them unite as the pressure falls. It is therefore important to get as much of the substances containing oxygen and hydrogen

in proportions, to form water, or approximate proportions, into the powder as possible, and I therefore prefer the baked wood, which contains these gases in such proportions, besides having its carbon, as stated, in a form to unite readily with oxygen. The fibrous character of my baked wood also gives toughness to the grains of powder and prevents the grains from breaking up too rapidly.

10 It is unnecessary to describe the method of combining the components of powder, for that is well known, but I have found the following ingredients and proportions to form a desirable powder for guns of twelve-inch caliber: 15 saltpeter, seventy-eight parts, by weight; sulphur, three parts; baked wood, 12.5 parts; ordinary wood pulp, 2.5 parts; sugar, (the use of which forms the subject of my application for Letters Patent filed August 12, 20 1885, No. 174,214,) four parts; or, as I have also found, the wood pulp may be omitted, as the grain will be toughened by the fiber of the baked wood, the proportions in this case being

about as follows: saltpeter, 78.95 parts, by weight; sulphur, three parts; baked wood 25 15.02 parts; sugar, 3.03 parts.

I do not limit myself to the special ingredients or proportions given above, as my invention consists in the combination of baked wood, as herein described, with well-known 30 gunpowder ingredients, and other equivalent ingredients may be substituted for those above mentioned.

What I claim is—

An explosive compound consisting of a nitrate and sulphur combined with charcoal retaining its fibrous structure, substantially as described. 35

In testimony whereof I affix my signature, in presence of two witnesses, this 15th day of June, 40 1886.

EUGENE DU PONT.

Witnesses:

WILLIAM H. BERRIGAN,  
THOMAS HUNT.